

## UNITED STATES PATENT OFFICE

2,132,724

PLASTICIZER AND PROCESS OF PRODUCING  
SAMEHarold R. Dalton, Teaneck, N. J., assignor to John  
S. Ware, New York, N. Y., Joseph F. Leete,  
Chappaqua, N. Y., and himselfNo Drawing. Application December 9, 1936,  
Serial No. 114,927

4 Claims. (Cl. 91—68)

This invention relates to plasticizing agents of the saccharide type, and to the method of producing same.

One object of the invention is to produce a plasticizing agent of this nature which is highly efficient, inexpensive to manufacture and which produces permanent plasticizing effects.

Another object of the invention is to produce such a plasticizing agent which comprises a water solution of a saccharide or combination of saccharides and reduction products of these saccharides such as sorbitol, mannitol, glycol, etc.

A further object of the invention is the provision of a method of producing such a plasticizing agent which consists of partially reducing a water solution of invert sugar to the state wherein it is broken up into water, invert sugar, sorbitol, mannitol and other reduction products.

Other objects and advantages of my improved plasticizing agent and the method of producing same will become more apparent as the description proceeds.

The disclosure made the basis of exemplifying the present inventive concept suggests a practical embodiment thereof, but the invention is not to be restricted to the exact details of this disclosure, and the latter, therefore, is to be understood from an illustrative, rather than a restrictive standpoint.

At the present time the use of a water solution of invert sugar as a plasticizer in the manufacture of paper, flexible glue and products such as gaskets and adhesives for gummed paper which employ glue in their manufacture, does not give altogether satisfactory results unless a small percentage of some other material is used along with it. The chief reason for this failure of water solutions of invert sugar to act as a satisfactory plasticizer results from their inability to remain in a physically stable state. Invert sugar when used either in paper or products of the type mentioned above will have crystals of dextrose slowly separate from it. In the case of paper plasticized with invert sugar this crystallization becomes apparent after the paper has aged for some time at relative humidities below 50%, in which case the paper gradually loses its flexibility and becomes brittle. Also paper which has had too much moisture removed from it during drying on the paper machine, will come off the machine in a brittle condition as a result of the crystallization of the dextrose. In the case of glue products this crystallization proceeds at relative humidities as high as 65%. In a flexible glue the crystals very quickly cover the surface of the material and

gradually penetrate through the entire mass. Here again the crystallization is accompanied by increasing brittleness. In the case of glue products which have become brittle as a result of the crystallization of the dextrose, conditioning at high relative humidities has little effect in bringing them back to their original state.

The above mentioned crystallization may be overcome by the addition of 20% to 30% of glycerine, by weight, to an invert sugar solution containing 77½% invert sugar (dry weight). Ethylene glycol in some cases is substituted for the glycerine. When using ethylene glycol, the percentage may vary somewhat from the 20% to 30% ratio found necessary when glycerine is used. Such additions, however, increase the cost of the product.

Since water solutions of invert sugar are not satisfactory in themselves for producing lasting and satisfactory plasticizing effects, I carried on extensive investigations as to the best manner of treating such solutions so that they may be modified for satisfactory use as a plasticizer.

The aforementioned investigations resulted in the development of a partially reduced invert sugar solution which gave highly satisfactory results when used as a plasticizer. This plasticizer, which will hereafter be termed partially reduced invert sugar plasticizer, was readily and economically prepared by the two methods described below:

1. *Reduction with sodium amalgam.*—A water solution of invert sugar containing 76.0% invert sugar by weight was treated with 2½% sodium amalgam. Equal weight of amalgam and invert sugar solution were used. The amalgam was added in small quantities. The reaction mixture was vigorously and continuously stirred until all of the amalgam was used up. The temperature of the mixture was maintained at 30° C. by placing the container in a water bath regulated to maintain this temperature. Sulphuric acid was added in small portions during the reaction in order to maintain the mixture neutral. The yield of reduced material was approximately 7.0%.

2. *Reduction with nickel in an atmosphere of hydrogen.*—A water solution of invert sugar containing 77.0% invert sugar by weight was placed in an autoclave containing catalytic nickel. The air was swept out of the chamber with hydrogen. The hydrogen pressure in the autoclave was finally raised to 1500 lbs./sq. in. The mixture in the autoclave was stirred for four hours, the pressure of hydrogen being maintained at 1500 lbs./

sq. in. and the temperature at approximately 35° C.

The catalytic nickel was prepared from nickel formate reduced with hydrogen at 300° C.

3 The yield of reduced material was approximately 25%, consisting principally of sorbitol and mannitol.

Other methods of reduction such as electrolytic and those employing zinc, magnesium, etc. can 10 be used in place of the foregoing.

By modifying the temperature and pressure in the second method described above large yields 15 of other reduction products beside sorbitol and mannitol, such as glycerol and glycols can be obtained which tend to improve the properties of the plasticizer.

I have found that by using the entire partly reduced mixture, comprising invert sugar, water, and the reduced material, as obtained by the 20 aforementioned process, as a plasticizer for paper, glue products and the like, the said products will be maintained in a stable plasticized state, and no tendency to become brittle will occur. I have also found that in a plasticizer 25 suitable for commercial use the ingredients may vary about as follows:

Invert sugar, glucose or fructose, etc., from a minimum of 50% to a maximum of 75%; water from a minimum of 10% to a maximum of 30% 30 and reduced materials (mixture of sorbitol, mannitol and other reduced products) from 5% to 30%.

Partially reduced invert sugar plasticizer of a composition falling within the above range of 35 compositions can be made by a slight variation of the method described. Thus glucose, fructose, xylose, sorbose, mannose, arabinose, etc., may be reduced by either of the methods described above and to the reduced product sufficient invert sugar 40 added to give a composition falling within the range specified.

A polysaccharide, like cane sugar (sucrose) or molasses, may be used as a starting material, inversion and reduction being made to take place 45 simultaneously. In this method the plasticizer may contain a small percentage of cane sugar.

As a final method of preparation, sorbitol and mannitol, which will contain other reduction products, may be isolated from a reduced sugar 50 mixture and added to an invert sugar solution to give a solution having a composition falling within the above mentioned range.

A highly satisfactory plasticizer made in accordance with my invention would comprise the 55 following ingredients in about the proportions specified:

|                   | Per cent |
|-------------------|----------|
| Invert sugar      | 50       |
| Water             | 25       |
| Reduced materials | 25       |

It is also possible to produce a satisfactory plasticizer by the addition of 25 lbs. of a mixture of commercial sorbitol and mannitol to 75 lbs. of invert sugar.

In producing sorbitol and mannitol commercially, it is possible that certain aforementioned reduction products may not be present in the commercial product, but I find that in my product these materials contribute greatly to the 5 production of a more efficient plasticizer.

I have found that it is more economical to produce the sorbitol and mannitol directly in the invert sugar in about the proportions indicated, than to independently produce and refine each 10 constituent and subsequently mix them.

I also find that a mixture such as mentioned above will make a more efficient plasticizer because it produces more stable and more lasting results when used as a plasticizer for paper, 15 fabrics, glue and the like. This is particularly true when compared with the usual mixture of invert sugar and glycerine which is a common compound for such purposes.

Wherever in the specification and in the claims 20 I have used the term "invert sugar", I desire it understood that any mono-saccharide is to be included.

Having described my invention, what I claim as new and desire to secure by Letters Patent is: 2

1. A plasticizer for paper and the like comprising a water solution of invert sugar, and the reaction products formed by partially reducing a water solution of invert sugar, said reaction products including sorbitol and mannitol, the 3 ratio by weight of the invert sugar to the reaction products being approximately as 2 is to 1, said reaction products serving to prevent crystallization of the un-reduced sugar.

2. A plasticizer for paper and the like comprising a water solution of invert sugar, and the reaction products formed by partially reducing a water solution of invert sugar, said reaction products including sorbitol and mannitol, the ratio by weight of the various ingredients being 4 approximately as follows: invert sugar 50 per cent, reaction products 25 per cent, water 25 per cent.

3. As a new article of manufacture, fibrous material impregnated and plasticized with a 4 water solution of invert sugar in major proportion and the reaction products formed by partially reducing the water solution of invert sugar, said reaction products including sorbitol and mannitol, and said reaction products being in 5 sufficient amount to prevent crystallization of the un-reduced sugar.

4. As a new article of manufacture, paper impregnated with a water solution of invert sugar and the reaction products formed by partially 5 hydrogenizing a water solution of invert sugar, said reaction products including sorbitol and mannitol, the ratio by weight of the various ingredients being approximately as follows: invert sugar 50 per cent, reaction products 25 per cent, 6 water 25 per cent.

HAROLD R. DALTON.